

# UNITED STATES PATENT OFFICE.

HUGH S. FOOTE, OF PITTSBURGH, PENNSYLVANIA, ASSIGNOR TO STANDARD CHEMICAL COMPANY, OF PITTSBURGH, PENNSYLVANIA.

## ALLOY.

1,366,254.

Specification of Letters Patent. Patented Jan. 18, 1921.

No Drawing.

Application filed September 29, 1920. Serial No. 413,526.

To all whom it may concern:

Be it known that I, HUGH S. FOOTE, a citizen of the United States, and a resident of Pittsburgh, in the county of Allegheny and State of Pennsylvania, have invented certain new and useful Improvements in Alloys; and I do hereby declare the following to be a full, clear, and exact description of the invention, such as will enable others skilled in the art to which it appertains to make and use the same.

This invention relates to improvements in steel alloys,—one object of the invention being to produce an alloy which shall have high static and dynamic strength, ductility and hardness without possessing the quality of so-called "high-speed" steel used in the manufacture of cutting tools, but which shall be eminently efficient when employed for making such devices as automobile gears and springs, light armor plate, rivet sets and other articles which are required to possess high static and dynamic strength, ductility and hardness and which do not have to perform functions of edged tools.

With this and other subjects in view, the invention consists in an alloy as hereinafter described and pointed out in the claims.

The ingredients which I employ alloyed with steel and the relative approximate proportions of said ingredients in the finished steel alloy are as follows:—

|            | Per cent.    |
|------------|--------------|
| Carbon     | 0.10 to 0.60 |
| Uranium    | 0.20 to 1.00 |
| Manganese  | 0.50 to 0.60 |
| Nickel     | 2.00 to 3.50 |
| Silicon    | 0.55 to 2.00 |
| Phosphorus | .03          |
| Sulfur     | Trace.       |

In making my improved steel alloy I may

first melt, in an electric furnace, a quantity of steel turnings under a slag of lime and iron scale and then slag and refine the metal under a basic carbid slag. The alloying elements manganese, nickel and silicon are added in the furnace,—the manganese and silicon thus added being in the form of ferro-manganese and ferro-silicon, and the uranium in the form of ferro-uranium may be added in the ladle.

My improved steel alloy, while not possessing the quality of so-called "high-speed" steel for use in making edged tools, it does possess in a very high degree, qualities of static and dynamic strength, ductility and hardness which render it eminently efficient and useful for the manufacture of such articles, for example, as automobile gears, light armor plate, rivet sets, etc.

Having fully described my invention, what I claim as new and desire to secure by Letters-Patent, is:—

1. An alloy consisting of steel having alloyed therewith, uranium, silicon and nickel in the proportions substantially as specified.

2. The herein described uranium-silico-nickel-steel alloy having uranium, silicon and nickel alloyed in the relative proportions substantially as specified with the steel, said alloy also containing carbon and manganese in the relative proportions substantially as specified.

In testimony whereof, I have signed this specification in the presence of two subscribing witnesses.

HUGH S. FOOTE.

Witnesses:

LILLIAN GANLEY,  
JAMES C. GRAY.